

## UNITED STATES PATENT OFFICE

2,256,614

## CAST ARTICLE

Russell Franks, Niagara Falls, N. Y., assignor to  
Electro Metallurgical Company, a corporation  
of West Virginia

No Drawing. Application June 7, 1940,  
Serial No. 339,327

4 Claims. (Cl. 75—128)

The invention relates to steels of the austenitic chromium-nickel type and refers more particularly to cast articles composed of such steels.

Austenitic chromium-nickel steels containing about 20% to 30% chromium, 5% to 25% nickel, and up to 1% carbon are widely used in the cast condition for high temperature service. For some conditions of service the cast steel used may contain other alloying elements in addition to chromium and nickel. Thus, where resistance to intergranular deterioration at carbide precipitation temperatures is necessary, the steels commonly contain columbium in a proportion of 4 to 12 times the carbon content, or titanium in a proportion of 2 to 10 times the carbon content, and where increased strength at elevated temperatures or increased resistance to specific corrodants is desired, the steels may contain 0.5% to 3.5% molybdenum. Manganese is often added in a proportion up to about 1%, and also nitrogen, to improve the quality of the steels.

As-cast steels of the composition described, are well suited in most respects to their use in high temperature service. They are resistant to many corrosive media and are adequately strong at moderately low temperatures. However, their ductility is poor at high temperatures between about 500° C. and 900° C. A cast tube or other vessel may to all outward appearances be in perfect condition yet fail suddenly without warning. The failure is not preceded by bulging or elongation such as usually precedes failure of ductile materials under stress.

This tendency of the cast chromium-nickel steels to fail at high temperature without warning is a disadvantage. While the length of life of articles composed of such steels may be entirely satisfactory, sudden failure of a part of an apparatus is dangerous to health and property. As a result, prudence requires frequent inspection and replacement long before the full life of the cast steel has been utilized.

It is a principal object of this invention to improve the ductility of cast austenitic chromium-nickel steels at high temperatures and thereby to prevent sudden, unexpected failure of such articles during use. This object is achieved by the addition of 1% to 6% manganese.

The invention accordingly comprises a cast article composed of austenitic chromium-nickel steel containing between 20% and 30% chromium, 5% to 25% nickel, 0.15% to 1% carbon, a substantial proportion not exceeding 5% of at least one ferrite-promoting element of the group consisting of titanium, columbium, and molybdenum, and 2% to 6% manganese, a proportion of manganese sufficient to impart to the steel improved ductility persisting at high temperatures. A preferred embodiment of the invention

is a cast vessel for use at high temperatures, for example, a tube.

The proportion of manganese included in austenitic steel according to this invention is not dependent on the proportion of nickel in the steel. Thus, for a steel containing 24% chromium and 12% nickel the optimum proportion of manganese is about 4%, and the same proportion of manganese is equally effective in a steel containing 25% chromium and 20% nickel.

The carbon content of steels to which manganese may be added to secure the benefits of increased ductility should not exceed 1% and preferably should be less than 0.5%. Nitrogen in a proportion between 0.01% and 0.5% may be substituted for part of the carbon to improve the strength of the steel; the proportion of nitrogen is preferably between 0.1% and 0.3%.

Short time high temperature tensile tests on steels of various compositions illustrate the usefulness of the invention. In making these tests cast samples of the different steels, machined to standard (A. S. T. M.) 0.505 inch diameter tensile test specimens, were gradually brought to a temperature of 870° C. and held for approximately one-half hour at that temperature. The samples were then transferred to a standard tensile test machine equipped with a heated muffle for maintaining the sample at temperature throughout the test, and tensile stress was gradually applied until the sample failed. After each test the sample was removed from the testing machine and allowed to cool to room temperature. The elongation and reduction of area of each sample were measured after cooling. Results of such tests are given in the following table. "T. S." means ultimate tensile strength in pounds per square inch, "Per cent El" means percentage elongation in two inches, and "Per cent R. A." means reduction in area.

## Tests at 870° C. on cast Cr-Ni steels

| Steel | Analysis (rest Fe) |             |            |             | Tensile test results |             |                |
|-------|--------------------|-------------|------------|-------------|----------------------|-------------|----------------|
|       | Per cent Cr        | Per cent Ni | Per cent C | Per cent Mn | T. S.                | Per cent El | Per cent R. A. |
| 1     | 24.90              | 11.94       | 0.40       | 0.75        | 24,400               | 17          | 27             |
| 2     | 25.25              | 11.75       | 0.36       | 2.01        | 23,600               | 19          | 34             |
| 3     | 25.00              | 12.04       | 0.39       | 4.14        | 20,500               | 35          | 58             |
| 4     | 24.52              | 11.86       | 0.43       | 6.03        | 21,000               | 27          | 54             |
| 5     | 25.30              | 10.76       | 0.24       | 0.84        | 18,260               | 18          | 21             |
| 6     | 25.06              | 10.79       | 0.24       | 2.04        | 19,400               | 27          | 39             |
| 7     | 24.80              | 10.89       | 0.23       | 3.83        | 18,700               | 30          | 52             |
| 8     | 24.80              | 12.02       | 0.22       | 3.89        | 16,150               | 39          | 77             |
| 9     | 25.30              | 12.09       | 0.26       | 3.99        | 25,900               | 31          | 33             |
| 10    | 24.20              | 20.37       | 0.24       | 5.59        | 19,300               | 25          | 56             |

<sup>1</sup> Contains 0.2 per cent nitrogen.

From the above table it is evident that the presence of manganese in cast chromium-nickel

steels materially benefits the ductility of such steels at elevated temperature.

While the invention is of particular value in its application to chromium-nickel steels containing between 20% and 30% chromium, it is also of benefit in austenitic chromium-nickel steels containing 10% to 20% chromium, 5% to 15% nickel, a substantial proportion not exceeding 5% of at least one ferrite-promoting element of the group consisting of titanium, columbium, and molybdenum, and 0.01% to 1% carbon. Preferably, the carbon is below 0.3%; a part of the carbon may be replaced by about 0.01% to 0.2% nitrogen. In steels containing 10% to 20% chromium the proportion of manganese which is of greatest benefit is between 1% and 4%, the optimum being about 2%.

Short time high temperature tensile tests made in the way explained above on representative chromium-nickel steels containing about 18% chromium and 8% to 10% nickel, and varying proportions of manganese illustrate the beneficial effects of manganese on ductility at high temperatures. Results of tests are given in the following table:

Tests at 870° C. on cast Cr-Ni steels

| Steel | Analysis (rest Fe) |            |           |            |            | Tensile test results |            |               |
|-------|--------------------|------------|-----------|------------|------------|----------------------|------------|---------------|
|       | Percent Cr.        | Percent Ni | Percent C | Percent Cb | Percent Mn | T. S.                | Percent El | Percent R. A. |
| 11    | 18.18              | 9.03       | 0.10      | None       | 0.49       | 17,000               | 21         | 41            |
| 12    | 18.04              | 9.15       | 0.10      | None       | 0.98       | 17,000               | 25         | 40            |
| 13    | 18.05              | 8.65       | 0.08      | None       | 1.60       | 14,550               | 39         | 72            |
| 14    | 18.15              | 10.05      | 0.06      | 0.75       | 0.64       | 16,625               | 25         | 61            |
| 15    | 18.87              | 10.36      | 0.07      | 0.78       | 1.65       | 17,325               | 38         | 68            |
| 16    | 18.02              | 10.01      | 0.08      | 0.65       | 3.08       | 19,000               | 43         | 60            |

While specific examples have been given of particular applications of the invention, these examples are given merely to illustrate its principles, and the invention is not limited to or by such examples.

I claim:

1. A cast article for use at elevated temperatures and composed of an austenitic chromium-nickel steel containing 20% to 30% chromium; 5% to 25% nickel; a substantial proportion not exceeding 5% of at least one ferrite-promoting element of the group consisting of titanium, columbium, and molybdenum; carbon in a proportion between 0.01% and 0.5%; 0.01% to 0.5% nitrogen; and a proportion of manganese between 2% and 6%, effective to impart enhanced ductility at elevated temperatures to the article; remainder iron.

2. A cast article for use at elevated temperatures between about 500° C. and 900° C. and composed of an austenitic chromium-nickel steel containing 20% to 30% chromium; 5% to 25% nickel; 0.5% to 3.5% molybdenum; carbon in a proportion between 0.15% and 0.5%; 0.01% to 0.3% nitrogen; a proportion of manganese between 2% and 6%, effective to impart enhanced ductility at elevated temperatures to the article; remainder iron.

3. A cast article for use at elevated temperatures and composed of an austenitic chromium-nickel steel containing 10% to 20% chromium; 5% to 15% nickel; a substantial proportion not exceeding 5% of at least one of the ferrite-promoting elements titanium, columbium, and molybdenum; carbon in a proportion between 0.01% and 0.3%; 0.01% to 0.2% nitrogen; a proportion of manganese between 1% and 4%, effective to enhance the ductility of such article at elevated temperatures; remainder iron.

4. A cast article for use at elevated temperatures between about 500° C. and 900° C. and composed of an austenitic chromium-nickel steel containing 10% to 20% chromium; 5% to 15% nickel; 0.5% to 3.5% molybdenum; carbon in a proportion between 0.01% and 0.3%; 0.01% to 0.2% nitrogen; a proportion of manganese between 2% and 4%, effective to impart enhanced ductility at elevated temperatures to the article; remainder iron.